

Jan. 15, 1935.

R. A. HAYWARD

1,987,901

PAPER AND METHOD OF MAKING

Filed Sept. 6, 1932



BY

Ralph A. Hayward  
Chappell & Earl  
ATTORNEYS

INVENTOR

## UNITED STATES PATENT OFFICE

1,987,901

## PAPER AND METHOD OF MAKING

Ralph A. Hayward, Parchment, Mich., assignor  
to Kalamazoo Vegetable Parchment Company,  
Parchment, Mich.

Application September 6, 1932, Serial No. 631,794

13 Claims. (Cl. 92—40)

The main objects of this invention are:

First, to provide an improved paper which has a relatively small amount of fibrous stock or paper stock and at the same time is strong, opaque and well adapted for use in printing.

Second, to provide an improved paper which is particularly desirable for use in the making of waxed paper for wrappers and the like and is not rendered transparent by the wax.

Third, to provide an economical paper well adapted for printing.

Fourth, to provide a method of making paper which permits very rapid and economical production of paper having the advantages above set forth.

Fifth, to provide a method of making paper which may be practiced on paper making machines now in extensive use with comparatively slight modification or change in the structure thereof.

Objects pertaining to details and economies of my invention will definitely appear from the description to follow. The invention is defined and pointed out in the claims.

The manner of carrying out my invention is illustrated in the accompanying drawing, in which:

Fig. 1 is a conventional illustration of a paper making machine or apparatus embodying my invention.

Fig. 2 is an enlarged fragmentary view showing the relation of the apparatus which may be employed in practicing my invention or method to other parts of the paper making machine, such parts being shown conventionally.

Fig. 3 is an enlarged fragmentary view illustrating one step of my improved method, a web or sheet of paper greatly enlarged in thickness being shown in relation to the impregnating rollers.

In the accompanying drawing 1 represents the forming portion of a paper making machine, 2 a set of drying rollers, 3 a second set of drying rollers, and 4 a calender or stack of calendering rollers. The web of paper is indicated at 5.

In this machine or apparatus illustrated I interpose a coacting pair of pressure rollers 6 and 7 between the sets of drying cylinders or rollers 2 and 3, guide rollers 8 and 9 being associated with the rollers 6 and 7 to guide the web 5 between them.

The web of paper 5 is formed and dried to substantial dryness by the first set of drying cylinders 2. The sheet or web is then impregnated so as to fill the spaces or interstices between the

fibers with a filler. I have attempted to illustrate the sheet or web in Fig. 3 as being porous, which is its normal condition as coming from the drying cylinders 2, that is, there are substantial spaces or interstices between the fibers, and at 50 I have attempted to illustrate the portion of the web that has passed through the rollers as filled or impregnated so that the spaces between the fibers are closed and the sheet rendered opaque.

I have found very satisfactory a filler material consisting of gum arabic, glycerin, water and a pigment such as fine clay or lithophone combined into a paste-like colloidal solution. The gum arabic, glycerin and water may be combined in the proportion of 12 pounds of gum arabic, 12 pounds of glycerin, and 25 pounds water, which results in a water soluble varnish. The clay or lithophone is then ground into this vehicle into a stable suspended condition or colloidal solution. "Lithophone" is a trade name for a mixture of zinc sulphide and barium sulphate. When this material is used it is treated the same as the clay.

A starch or glucose vehicle may be employed instead of the gum arabic vehicle, the object being to provide some vehicle which will, with the pigment, form a colloidal solution.

This filler material is applied to both sides of the web just before it passes between the pressure rollers 6 and 7. A spray pipe 10 is shown above the web to discharge thereon while a spray pipe 11 is shown below to discharge upon the roller 7 by which it is carried up to the under side of the web so that, when the web passes between the rollers, it carries the filler material which is forced by the heavy pressure of the rollers between the fibers and very completely fills the spaces between the same. These rollers 6 and 7 should be of non-yielding material and I have successfully employed steel rollers.

As there are several thousand pounds pressure at the nip or bite point between the rollers and as the filler material is in a colloidal state it is not pressed out of the vehicle but is forced into the substantially dry web or sheet, very completely and effectively filling the same. The fiber is not displaced or broken so the full strength of the paper is retained. At the same time the sheet is rendered opaque and a good printing surface provided.

The sheet is especially desirable for use in the manufacture of waxed paper as the opaqueness is not destroyed by the application of the wax. Further, where a white pigment is used

the sheet is a clear white and is not discolored as sometimes results from the application of wax.

It is desirable that the sheet be substantially dry at the time of impregnation and it is then dried by passing through the second set of drying rollers. It may be calendered as part of a continuous paper making operation.

This method permits very high speed on the machine, as high as 800 feet per minute having been run with good results. This has not been found possible so far as I am aware in producing ordinary paper for fine printing.

The filler is forced into the web, or the web is impregnated, as distinguished from a surface coating such as is commonly employed on "book" papers.

It will be understood that my improved paper is not designed or intended to have all the qualities of coated paper as the ordinary coated paper has a surface coating, whereas, my paper is impregnated with a material that fills the interstices thereof without dislocating or destroying the fibers. As stated, the paper is highly desirable as an economical printing paper and is especially desirable for waxing.

Having thus described my invention what I claim as new and desire to secure by Letters Patent is:

30. 1. The method of making paper consisting of forming and drying the web, applying a filler material in colloidal suspension to both sides of the web, and passing the web between non-yielding pressure rollers whereby the filler material is forced into the interstices between the fibers and filling and impregnating the same throughout.

40. 2. The method of making paper consisting of forming the web, drying, and applying a filler material in colloidal suspension to the web and forcing the filler into interstices between the fibers and substantially filling and closing the same by rolling contact pressure.

45. 3. The art of making paper consisting of applying a filler material in colloidal suspension to both sides of a dry sheet or web, passing between nonresilient pressure rolls whereby the filler material is forced into the interstices of the sheet or web and filling and impregnating the same throughout.

50. 4. The method of making paper consisting of forming and drying the web, applying a colloidal solution consisting of gum arabic, glycerin and water and a pigment to both sides of the web and then passing the web between non-yielding pressure rollers whereby it is subjected to high pressure, drying, and calendering.

55. 5. The method of making paper consisting of forming and drying the web, applying a colloidal

solution consisting of gum arabic, glycerin and water and a pigment to both sides of the web and then passing the web between non-yielding pressure rollers, whereby it is subjected to high pressure.

5

6. The art of making paper consisting of applying a filler in colloidal suspension to both sides of a dry sheet or web, and passing between non-resilient pressure rollers whereby the filler is forced into the spaces between the fibers and filling such spaces and impregnating the sheet throughout.

10. 7. The art of making paper consisting of applying filler material in colloidal suspension to a dry sheet or web and forcing the material into the spaces between the fibers and filling the same, drying and calendering.

15. 8. The art of making paper consisting of applying filler material in colloidal suspension to a dry sheet or web and forcing the material into the spaces between the fibers filling and impregnating the same, and drying.

20. 9. The art of making paper consisting of forming a web and drying, and applying a filler in colloidal suspension and forcing such material into the sheet or web under high pressure 25 until the pores or spaces between the fibers are filled and impregnated by the filler.

25. 10. The art of making paper consisting of applying a filler in colloidal suspension to a formed 30 dry sheet or web and forcing such filler into the sheet or web under high pressure, thereby filling and impregnating the spaces between the fibers.

35. 11. The art of making paper consisting of impregnating a formed dry sheet or web with a filler consisting of gum arabic, glycerin and water and a pigment combined into a colloidal solution, the solution being forced into and impregnating the spaces between the fibers of the 40 sheet by pressure.

45. 12. The art of making paper consisting of filling the spaces between the fibers of a formed dry sheet or web with a colloidal solution consisting of gum arabic, glycerin and water and a pigment.

50. 13. In the art of making substantially opaque paper which retains its opacity even when waxed, the steps which comprise passing a web of paper, formed of sulphite stock, through a series of drying rolls; applying colloidal material to both sides of the dry web; then passing the web between a pair of non-yielding steel rolls under high pressure, whereby the colloidal material is forced into the fibers of the paper, substantially closing all spaces or openings between the fibers; and finally passing the web through a series of drying rolls.

RALPH A. HAYWARD.